

March 29, 1949.

J. B. MORTON

2,465,467

ELECTRIC BLASTING CAP

Filed June 11, 1946



FIG. 1



FIG. 2

JOHN B. MORTON  
INVENTOR.

BY

*Ernest G. Peterson*

AGENT

## UNITED STATES PATENT OFFICE

2,465,467

## ELECTRIC BLASTING CAP

John B. Morton, Hopewell, Va., assignor to Hercules Powder Company, Wilmington, Del., a corporation of Delaware

Application June 11, 1946, Serial No. 675,865

10 Claims. (Cl. 102—28)

1

This invention relates to an improved electric blasting cap and, more particularly, to a safety-type electric blasting cap.

It is well known that an electric blasting cap of the safety type may have a base charge comprising a secondary explosive and a priming charge superimposed thereon comprising an explosive of the so-called safety type, such as the nitrated saccharides, nitromannite and nitrolactose. These priming charges are ignited by means of a deflagratable composition or by means of a semi-explosive burst from a match-head-type assembly superimposed thereon. These caps are known to be less sensitive toward detonation upon the application of strong external heat than similar blasting caps having a primary charge comprising such explosives as mercury fulminate, diazodinitrophenol, lead azide, etc. Safety-type electric blasting caps have several disadvantages, one being that the ignition charge necessary to set off the safety-type primary charge must have unusually strong ignition characteristics, another being that the priming charge requires an added confinement comprising a reinforcing capsule or inner shell in order to be fully effective, and still another is that, in most instances, relatively greater amounts of the safety-type priming charge must be used in order to effect proper detonation of the base charge.

Now in accordance with the present invention it has been discovered that when a high heat-stable primary charge of lead azide is positioned centrally and in the upper portion of a heat-unstable priming or explosive charge, such as nitrolactose which is in turn superimposed upon a base charge, the disadvantages found with prior art safety-type electric blasting caps are eliminated.

It is an object of this invention to provide an electric blasting cap which may be heated externally to a high temperature without causing detonation.

Another object of this invention is to provide a safety-type electric blasting cap that is simple in construction, economical to manufacture and reliable.

Other objects of the invention will appear hereinafter, the novel features and combinations being set forth in the appended claims.

Preferred embodiments of this invention have been chosen for the purpose of illustration and description and are shown in the accompanying drawing, forming a part of the specification wherein:

Fig. 1 is an elevational view in partial section

2

of the electric blasting cap in the course of construction; and

Fig. 2 is an elevational view in partial section of the completed cap.

5 An improved electric blasting cap was manufactured in accordance with the present invention by placing a base charge 1 comprising 0.20 gram of tetryl into a shell 2 of 0.30-inch inside diameter, and pressed with a flat pin under a pressure of 4000 pounds per square inch. A heat-unstable priming charge 3, consisting of 0.12 gram of nitrolactose, was superimposed on top of the tetryl base charge and pressed with a step-cut pin 4 under a pressure of 200 pounds per square inch. 10 The use of the step-cut pin, shown in Fig. 1 being withdrawn from the shell 2, forms a cavity 5 centrally located in the priming charge 3 and located in the upper portion thereof. The dimensions of the cavity 5 may be changed in such 15 a way as to vary the depth to which the cavity extends into the priming charge 3, depending upon the length of the column of priming charge being used. The cavity is positioned as near the center of the priming charge as is possible so 20 as to provide the maximum amount of insulation and cushioning by that portion of the priming charge 3 indicated by the numerals 6 for a given amount of heat-stable primary charge.

A heat-stable primary charge 7 comprising 0.02 25 gram of lead azide is charged into the minimum volume cavity 5 after which the ignition charge and the priming charge are pressed simultaneously with a flat pin under a pressure of 2000 pounds per square inch. A bridge assembly, comprising a plug 8 having a cavity 9 at the lower end thereof and a pair of spaced leg wires 10 extending therethrough and terminating adjacent the cavity 9 in a pair of bridge wire supports connected by a bridge wire 11, is moved into 30 the open end of the shell 2. The cavity 9 was previously filled with an ignition charge 12 consisting of 19.0% diazodinitrophenol, 65.8% potassium chlorate, 13.2% charcoal, and 2.0% nitro-starch. Thus, the ignition charge is placed in 35 juxtaposition to the primary charge as shown in Fig. 2. The shell was then closed against moisture with a waterproofing compound 13 and a sealing compound 14.

Electric blasting caps prepared in accordance 40 with the above example give an excellent lead plate test in accordance with the standards set up by the U. S. Bureau of Mines.

Electric blasting caps prepared in accordance 45 with the above example were tested to determine their sensitivity to ignition from extreme heat by

placing the caps in a molten metal bath at various temperatures. The results of these tests are given in the table, column 1.

More electric blasting caps were made similar to the above example, except that the heat-stable primary charge, lead azide, was positioned in a layer over the entire top surface of the priming charge which consisted of 0.22 gram of nitrolactose. These caps were also subjected to the same molten metal bath test and the results are given in column 2 of the table. Five caps of each type were tested at the temperature given in the table.

10

weight of nitrolactose and lead azide being used. For example, when 0.15 gram of nitrolactose is used, 0.01 gram of lead azide centrally positioned on the top side of the priming charge will effect proper detonation of the base charge. When 0.10 gram of nitrolactose is used, 0.02 gram of lead azide is necessary, and, when 0.05 gram of nitrolactose is used, 0.14 gram of lead azide is necessary.

10 The ignition mixture contained in the cavity 9 of the plug assembly may be any of the compatible conventional ignition mixtures used in

TABLE  
*Behavior of electric blasting caps in molten metal bath*

| Temperature | Column 1                                        |     | Column 2                                                      |     |
|-------------|-------------------------------------------------|-----|---------------------------------------------------------------|-----|
|             | Time for Decomposition, Sec.                    | Av. | Time for Decomposition, Sec.                                  | Av. |
| 372° F      | 74, 62, 64, 71, 72                              | 69  | 44, 64, 62, 60, 52                                            | 56  |
| 390° F      | 45, 53, 61, 62, 48                              | 54  | 55, 43, 39, 52, 40                                            | 46  |
| 405° F      | 38, 29, 30, 31, 39                              | 33  | 29, 33, 26, 37, 35                                            | 32  |
| 419° F      | 23, 1 <sup>2</sup> 25, 2 <sup>1</sup> 31, 32, 8 | 24  | 20, 28, 27, 7, 1 <sup>2</sup> 9                               | 18  |
| 433° F      | 27, 25, 25, 6, 20                               | 21  | 7, 8, 1 <sup>2</sup> 7, 6, 2 <sup>1</sup> 10                  | 7   |
| 446° F      | 4, 4, 3, 1, 2 <sup>1</sup> 7                    | 4   | 4, 2 <sup>1</sup> 1, 2, 2 <sup>2</sup> 2, 4                   | 3   |
| 472° F      | 3, 4, 3, 4, 2                                   | 3   | 2, 1 <sup>2</sup> 1, 2, 2 <sup>1</sup> 2, 2 <sup>2</sup> 1, 1 | 2   |

Total partial shots, column 1, 2; column two, 6. Total complete shots, column one, 2; column two, 5.

<sup>1</sup> Partial shots.

<sup>2</sup> Cap detonated completely. In all other cases, caps puffed without violence.

It is noted that the tendency toward detonation with increased external heat is less pronounced with caps in which the lead azide is centrally positioned on the top side of the priming charge than with caps in which the lead azide is positioned over the entire top surface of the priming charge. The charges in which the lead azide was centrally positioned were decomposed at a slower rate than those in which the lead azide was positioned over the entire top of the surface.

Tests of these two types of caps for purposes of determining the minimum priming charge necessary to detonate a base charge of tetryl indicate that, for a given amount of a priming charge of nitrolactose, a lesser weight of primary charge of lead azide is necessary when the lead azide is carried in a minimum volume cavity positioned centrally and on the top side of the priming charge than when the lead azide is spread in the form of a wafer over the entire top side surface of the priming charge.

Suitable safety-type priming charges operable in accordance with this invention are solid nitrated saccharides, such as, for example, nitrolactose, nitromannite, nitrosucrose, nitroinositol, etc.

Suitable base charges are any of the base charges commonly used in electric blasting caps such as, for example, tetryl, trinitrotoluene, nitrostarch, PETN, etc. The preferred combination of charges is a combination of charges wherein the base charge is tetryl, the priming charge is nitrolactose, and the primary charge is lead azide.

In U. S. Patent 1,928,207 to Large, it is shown that 0.05 gram of nitrolactose is necessary to detonate a tetryl base charge. The caps prepared in accordance with this invention use 42% less nitrolactose when combined with lead azide in the manner disclosed to effect the same desirable detonation of the base charge of tetryl. In accordance with this invention, the minimum priming charge necessary to detonate the tetryl will vary in accordance with the proportional

35 electric blasting caps where primary charges of lead azide, diazodinitrophenol, mercury fulminate, etc., are used. In contradistinction to the strong ignition charges necessary in order to properly ignite a safety-type electric blasting cap, the present invention provides for the use of the conventional and well-known types of ignition compositions in juxtaposition to the primary charge.

40 From the foregoing description, it is apparent that the objects of this invention have been accomplished by providing a safety-type electric blasting cap comprising a primary charge of lead azide positioned in a minimum volume cavity held in insulated and cushioned relationship with the shell of the detonator on the top side of a heat-unstable priming charge, whereby a minimum amount of priming charge is necessary in order to properly detonate the base charge.

45 What I claim and desire to protect by Letters Patent is:

1. An electric blasting cap having in combination a base charge, a heat-unstable priming 55 charge superimposed on the base charge, a primary charge of lead azide disposed centrally in the upper portion of the priming charge, and an ignition charge in juxtaposition to the primary charge.

2. An electric blasting cap having in combination a base charge, a priming charge of a solid nitrated saccharide superimposed on the base charge, a primary charge of lead azide disposed centrally in the upper portion of the priming charge, and an ignition charge in juxtaposition to the primary charge.

3. An electric blasting cap having in combination a base charge, a priming charge of nitrolactose superimposed on the base charge, a primary charge of lead azide disposed centrally in the upper portion of the priming charge, and an ignition charge in juxtaposition to the primary charge.

4. An electric blasting cap having in combination a base charge, a priming charge of ni-

tromannite superimposed on the base charge, a primary charge of lead azide disposed centrally in the upper portion of the priming charge, and an ignition charge in juxtaposition to the primary charge.

5. An electric blasting cap having in combination a base charge, a priming charge of nitro-sucrose superimposed on the base charge, a primary charge of lead azide disposed centrally in the upper portion of the priming charge, and an ignition charge in juxtaposition to the primary charge.

6. An electric blasting cap having in combination a heat-unstable explosive charge, a charge of lead azide disposed centrally in the upper portion of the heat-unstable explosive charge, and an ignition charge in juxtaposition to the charge of lead azide.

7. An electric blasting cap having in combination a heat-unstable explosive charge of a solid nitrated saccharide, a charge of lead azide disposed centrally in the upper portion of the heat-unstable explosive charge, and an ignition charge in juxtaposition to the charge of lead azide.

8. An electric blasting cap having in combination a heat-unstable explosive charge of nitrolactose, a charge of lead azide disposed cen-

trally in the upper portion of the heat-unstable explosive charge, and an ignition charge in juxtaposition to the charge of lead azide.

9. An electric blasting cap having in combination a heat-unstable explosive charge of nitromannite, a charge of lead azide disposed centrally in the upper portion of the heat-unstable explosive charge, and an ignition charge in juxtaposition to the charge of lead azide.

10. An electric blasting cap having in combination a heat-unstable explosive charge of nitro-sucrose, a charge of lead azide disposed centrally in the upper portion of the heat-unstable explosive charge, and an ignition charge in juxtaposition to the charge of lead azide.

15 JOHN B. MORTON.

#### REFERENCES CITED

The following references are of record in the 20 file of this patent:

#### UNITED STATES PATENTS

|    | Number    | Name     | Date           |
|----|-----------|----------|----------------|
|    | 1,928,208 | Large    | Sept. 26, 1933 |
| 25 | 2,086,532 | Burrows  | July 13, 1937  |
|    | 2,350,172 | Lawrence | May 30, 1944   |
|    | 2,402,235 | Burrows  | June 18, 1946  |

**Certificate of Correction**

Patent No. 2,465,467.

March 29, 1949.

JOHN B. MORTON

It is hereby certified that errors appear in the printed specification of the above numbered patent requiring correction as follows:

Column 3, line 67, for "0.05 gram" read *0.50 gram*; column 4, lines 68 and 69, for "nitrolacetose" read *nitrolactose*; and that the said Letters Patent should be read with these corrections therein that the same may conform to the record of the case in the Patent Office.

Signed and sealed this 30th day of August, A. D. 1949.

[**SEAL**]

THOMAS F. MURPHY,  
*Assistant Commissioner of Patents.*